

## UNITED STATES PATENT OFFICE

2,295,593

## YARN PREPARATION

John Blanchard Miles, Jr., Greenville, Del., assignor to E. I. du Pont de Nemours & Company, Wilmington, Del., a corporation of Delaware

No Drawing. Application July 30, 1941,  
Serial No. 404,621

9 Claims. (Cl. 57—140)

This invention relates to yarn preparation, and more particularly, it relates to a process for setting the twist in a yarn comprising filaments of a synthetic linear polymer of the type disclosed in Carothers U. S. Patent No. 2,071,250.

This invention will be described with particular reference to Nylon yarns, i. e., yarns comprising filaments of synthetic linear polyamides as disclosed in Carothers U. S. Patent No. 2,130,948 and U. S. Patent No. 2,071,253. Since, however, many of the other synthetic linear polymers disclosed in the above-mentioned Patent No. 2,071,250 are subject to the peculiar setting characteristics of Nylon and since they may also be advantageously processed in accordance with the present invention, the term "Nylon" is intended to include them as equivalents in the present invention.

The tendency of a twisted yarn to untwist is known as "twist liveliness" and renders a yarn difficult, if not impossible, to handle in subsequent textile operations. It is known that the tendency of a twisted yarn to untwist on handling may be reduced by subjecting the yarn to treatment under hot, wet conditions. It is also known that Nylon yarn, as well as yarn comprising other synthetic linear polymers disclosed in Patent No. 2,071,250, is responsive to twist-setting treatment under hot, wet conditions. For instance, it is disclosed in two Carothers patents, U. S. Patents Nos. 2,130,948 and 2,157,116, that the twist in a Nylon yarn may be set by treatment with steam.

Such previously known methods of twist-setting when applied to Nylon yarn, however, have the disadvantage that the treatment impairs the subsequent utility of the Nylon yarn. This is because, as is shown in Miles U. S. Patent No. 2,157,117, the treatment of a Nylon yarn with steam tends to impart a yarn-setting in the yarn as well as a twist-setting. A yarn that has been yarn-set will tend to retain the physical configuration that it had at the time of yarn-setting. That is, a yarn which was straight when steam-treated will tend to remain straight, a yarn which was looped will tend to remain in loops, etc. Since the yarn, after twist-setting, is usually knitted or woven into a fabric, the use of a yarn which has become yarn-set during the twist-setting will result in the production of a fabric having poor stitch or weave formation because of this wiry tendency of the yarn to resume the configuration it had at the time of yarn-setting. This phenomenon of yarn-setting does not take place in other natural and syn-

thetic yarns but seems to be specific to the above-mentioned synthetic liner polymer yarns, particularly Nylon yarns.

It is known that subjecting a twisted Nylon 5 yarn to hot, wet conditions which are not as drastic as the steam treatment will set the twist to a certain extent without yarn-setting. Such a process is disclosed in Miles U. S. Patent No. 2,157,119 in which it is shown that the twisted 10 yarn may be twist-set by exposing it, while wound on pins, to air at 170° F. and 78% relative humidity for one hour. In Sommaripa U. S. application, Serial No. 226,683, now U. S. Patent No. 2,251,962, there is disclosed a method of reducing the liveliness of a twisted sewing thread by allowing the thread, after twisting, to stand under the same conditions as in U. S. Patent No. 2,157,119. According to the standard practice in 15 twist-setting, the yarn in both these examples was treated while wound on a rigid support. However, the liveliness of the twist was not sufficiently reduced by this process for easy subsequent handling. This is shown in the Sommaripa patent where it is disclosed that the 20 twist so treated was too lively and that a further treatment with boiling water was necessary. Such treatment, of course, had the disadvantage of 25 yarn-setting.

Thus, it will be seen that a useful twist-setting 30 of Nylon yarns has, heretofore, presented a difficult problem. On the one hand, if the yarn is subjected to a steam treatment, although the 35 twist is set, yarn-setting also occurs. If, however, on the other hand, the package of yarn is subjected to somewhat milder conditions in order to avoid yarn-setting, the twist is not set 40 sufficiently and the yarn exhibits an unsatisfactory amount of twist liveliness. These difficulties are particularly increased when the twisted 45 yarn is of fine denier and highly twisted, and it is these Nylon yarns that have proved so advantageous in many textile uses, especially in the production of sheer, full-fashioned hosiery and crepe fabrics.

It is, therefore, an object of this invention to 50 provide a satisfactory process for setting a twist in Nylon yarn to substantially reduce twist liveliness without imparting to the yarn objectionable yarn-setting.

It is a further object of this invention to 55 provide a twisted Nylon yarn in which the twist liveliness has been reduced to a satisfactory degree without objectionably yarn-setting the same.

Other objects of this invention will appear hereinafter.

These objects are accomplished, in general, by the twist-setting of the yarn under mild, hot, wet conditions while permitting the yarn to shrink.

It has now been found that a Nylon yarn may be twist-set to very materially reduce its twist liveliness by subjecting the same to hot, wet conditions which are sufficiently mild to prevent objectionable yarn-setting if the yarn, during this processing, is maintained under a sufficiently relaxed condition to permit the same to shrink. Neither the twist liveliness nor the yarn-set in a yarn produced in this manner will objectionably interfere with its use in textile operations. It is not known whether the twist liveliness is reduced because of the effect of the hot, wet conditions or whether it is reduced because of the shrinkage that takes place in the yarn during this process. That the shrinkage is an important factor in reducing the twist liveliness of the yarn is shown by the fact that if the yarn is shrunk by any means before twisting, it is very difficult to set the twist later. Also, the residual shrinkage, that is, the shrinkage of which a yarn is capable after twist-setting, is proportional to the tension under which the yarn is kept while the twist-setting operation is being performed. Additionally, in any particular yarn, its residual shrinkage after twist-setting is directly proportional to its twist liveliness. That is, the lower the residual shrinkage of a twisted yarn, twisted from identical filaments, the lower the twist liveliness and thus the better twist-set the yarn.

In order that the process of this invention may be more clearly understandable the following examples are set forth, although it will be clearly understood that the invention is not limited to these specific embodiments.

#### Example I

Thirty-denier, 10-filament, unsized polyhexamethylene adipamide yarn which has been twisted to 30 turns per inch was wound into skeins and twist-set at 170° F. and 88% relative humidity for one and one-half hours while permitting the skeins to shrink freely without untwisting or snarling. These skeins were then allowed to dry and cool and the liveliness of the yarn tested. The twist liveliness before setting was 11.25 units and after treatment was found to be 0.5 unit, the yarn-set showed an angle of 75°, and the yarn was entirely satisfactory for further textile operations.

The twist liveliness referred to above is measured by means of a test which gives a quantitative measure of the liveliness of twisted yarn, i. e., the tendency or force with which the yarn tends to twist up on itself. The test is carried out as follows: One end of the yarn to be tested is held in a clamp on the end of a brass bar and the other end is held in another clamp which is movable so that it slides along the bar. In carrying out the twist liveliness test, the yarn is carefully clamped under just enough tension to keep it straight with the clamps 50 centimeters apart, care being taken not to back up the twist in the handling of the yarn. A weight of 0.5 gram is hung at the midpoint of the yarn free of the brass bar and subject to the influence of gravity. The movable clamp is then brought toward the fixed clamp and at a definite distance between the two ends of the yarn, the yarn begins

to twist up on itself. The distance between the two clamps, measured in centimeters, at the point where the yarn begins to twist up on itself, is taken as the measure, in units, of twist liveliness. Therefore, the smaller this distance, the lower is the unit value of twist liveliness and the better the twist-setting in the yarn.

This test was designed to measure the twist liveliness of yarns of the customary denier of sheer, full-fashioned hosiery, that is, from 20 to 50 denier. Obviously, it will be necessary to increase weight at the midpoint of the yarn when the test is applied to yarns of materially heavier denier.

The angular degree of yarn-set referred to throughout the specification and claims is measured in the following manner: The yarn to be tested is wound around a wedge-shaped blade having an angle of 23° so that the yarn is bent through an angle of 157°. The wedge carrying the yarn is immersed in boiling water for thirty minutes. This is a drastic setting treatment and will set the yarn to the degree that it was not yarn-set by the twist-setting operation. The yarn is then removed from the wedge by cutting and dried in a relaxed condition and the remaining angles are measured. If the inside angle remaining in the yarn is low, it would indicate that there had been little yarn-setting in the twist-setting operation. Similarly, if the inside angle remaining in the yarn is high, it would indicate that there had been much yarn-setting in the twist-setting operation. The angular degree of yarn-set imparted to a yarn which is subjected to a twist-setting operation should not exceed 120° when tested in the above-described manner. A yarn having yarn-set to exceed 120° will not be satisfactory for use in weaving or knitting processes. For yarns comprising very heavy denier filaments, the angular degree of yarn-set as measured in the manner described should preferably be materially less than 120°.

#### Example II

A polyhexamethylene adipamide yarn similar to Example I, except that it had been sized with a partially hydrolyzed polyvinyl acetate size containing boric acid and polyethylene oxide as disclosed in the copending application of Daniel E. Strain, Serial No. 357,755, filed September 21, 1940, was wound on a bobbin carrying a removable collapsible shell. After winding, the shell was removed and collapsed to permit the unrestrained shrinking of the yarn during twist-setting. This yarn was then twist-set under the same conditions and for the same length of time as in Example I, after which the liveliness was found to be 3.5 units, the yarn-set showed an angle of 75° and the knitting performance was satisfactory.

#### Example III

Thirty-denier, 10-filament polyhexamethylene adipamide yarn of 2 turns per inch twist was uptwisted with the addition of 29 turns twist. Between the balloon pigtail of the uptwister and the take-up bobbin, the yarn under a tension of 3 grams was passed through a moistening device and then through a slot 3 1/2 inches long in a copper block electrically heated to 115° C. This yarn after this treatment was found to have a twist liveliness of 3.1 units and a yarn-set of 100°. The yarn was subsequently coned and knit without difficulty because of liveliness.

*Example IV*

A 30-denier, 10-filament, 30-turn sized polyhexamethylene adipamide yarn in the form of a warp was moistened by means of a roller running in a trough of water. After this moistening, the warp was run through a heating tunnel at 105° C. This tunnel was 21 feet long and the yarn was run through it at a rate of 800 feet per minute under a tension of 14 grams. The twist liveliness of the resulting yarn was 3.4 units and it knit satisfactorily without kinking.

*Example V*

A 30-denier, 10-filament, 30-turn polyhexamethylene adipamide yarn which had been sized was twist-set on a rigid bobbin to which it had been wound under a tension of 18 grams. This yarn was twist-set for one and one-half hours under the conditions of 170° F. and 88% relative humidity. This yarn was found to have a twist liveliness of 5.5 units and was found to kink objectionably during knitting. A similar sample of sized yarn was wound to skeins and was twist-set under the same conditions as described above except that the skeins were free to shrink. The yarn was then found to have a twist liveliness of 2 units and the knitting performance was satisfactory. This example is included to show the difference between the twist liveliness of yarn which has been twist-set without permitting shrinkage and that where shrinkage is allowed.

Although this invention has been described in terms of specific examples, it will be readily understood that numerous modifications may be made while still remaining within the scope of this invention. In Examples I, II, and V, the conditions of twist-setting were 170° F. and 88% relative humidity. The optimum conditions for twist-setting in an atmosphere of elevated temperature and high relative humidity to obtain a low twist liveliness, according to this invention, lie between 170° and 190° F. with a relative humidity between 85% and 100%. However, twist-setting may be carried out to give a yarn which does not have excessive liveliness even if the temperature of setting is reduced as low as 135° F. To achieve satisfactory results, the relative humidity of the atmosphere of twist-setting must be maintained above 50% and it is preferred to operate with a humidity above 75%. Instead of subjecting the yarn to atmospheric conditions of high temperature and high humidity, it may be subjected to water having a temperature of between 135° F. and 190° F. A temperature in excess of 150° F. is preferred. Of course, it will be readily understood that if the twist-setting conditions are made too drastic, yarn-setting will result; consequently, the twist-setting should not be carried out at a temperature in excess of 190° F. The temperature used will depend, to some extent, upon the time of treatment and the weight and particular character of the Nylon yarn. It is important that the exposure to these conditions be maintained long enough so that all of the underlying layers of yarn be exposed to the hot, wet conditions. The time and temperature employed in the treatment may be readily determined by the above-described twist-setting and yarn-setting tests.

It will be obvious, of course, that the heat may be provided in any one of several ways. For example, hot water, steam, heated air, heated metal plates, infra red, hot gases or vapors, warm alcohol or similar swelling agents may be used.

Although this invention has been described in the examples in terms of twist-setting of 30-denier yarn which has been twisted to 30 turns per inch, the method of the present invention is applicable to yarns of different deniers and degrees of twist. Other things being equal, it is obvious that twist liveliness will vary with the helix angle of the twist in the yarn. It will also be readily apparent that the method of this invention is of no importance unless the yarn has sufficient twist to give trouble, in a textile operation, from twist liveliness.

The degree of twist in a yarn of a given diameter is determined by the number of turns per inch. The degree of twist in yarns of different diameters is determined more accurately by the "helix angle" of twist as described in "An Introduction to the Micro-Analysis of Yarn Twist" by E. R. Schwarz, published in the "Journal of the Textile Institute" for March, 1933. The present invention is applicable to reduce twist liveliness in Nylon yarns having on the basis of the yarn diameter, a minimum twist commensurate to a 20-turn per inch twist in a 30-denier yarn.

Heretofore, particular difficulty has been encountered from the twist liveliness of yarns having a very high twist, for example, a crepe Nylon yarn of 30 denier having a twist of 50 turns per inch. The principles of the present invention can be utilized in setting the twist in such a yarn by first twisting the same to a greater extent than required, twist-setting in accordance with the present invention and then back-twisting to the desired twist. For example, to produce a 30-denier, 50-turn yarn, the yarn can be twisted to 55 turns per inch, twist-set and then back-twisted 5 turns per inch. The resulting yarn will not have an objectionable twist liveliness.

In order that shrinkage may be allowed while the twist-setting process is going on, it is necessary that the tension of the yarn during twist-setting be kept below certain limits. It has been found that the residual shrinkage of a twist-set yarn varies in direct proportion with the tension to which it was subjected while being twist-set. Since the twist liveliness of the yarn is proportional to the residual shrinkage, it will be readily seen that the twist liveliness will be proportional to the tension during twist-setting. In order that twist liveliness be reduced to a satisfactory degree, the tension during twist-setting should not exceed 0.66 gram per denier and it is preferred that the tension not exceed 0.4 gram per denier. As for the lower limit of tension, it is only necessary that sufficient tension be applied to the yarn to prevent it from looping back during setting. This may easily be determined by one skilled in the art.

As is shown in the examples, this process may be carried out either while the yarn is stationary or moving. The twist-setting may be performed when the yarn is loosely held in skeins with only sufficient tension to prevent looping or it may be loosely wound on a bobbin. Also, a collapsible bobbin may be used as shown in Example II. It is sometimes advantageous to perform the twist-setting operation while the yarn is traveling from one package to another or while in a warp as in Examples II, III and IV. In certain instances, twist-setting may be carried out in conjunction with the sizing operation so that, after the yarn is sized, it can then be twist-set while still on-the-run before winding up. Of course, the twist-setting step can be car-

ried out in two or more stages prior to the textile operation. For example, in the orderly operation of a plant, there may not be sufficient time to carry out fully the twist-setting on a size bobbin but there may be time available during the subsequent coning operation. In such a case, the twist-setting operation may be carried out in both places for suitable periods of time. As is shown in the examples, this process is, of course, applicable to both sized and unsized 10 yarns.

It is also within the scope of this invention to twist-set a yarn while allowing only partial shrinkage so that some twist-setting takes place and the yarn is also capable of further shrinkage. Although this will give a more lively yarn, in certain textile purposes such a yarn may be used to advantage. A yarn which has been twist-set while allowing partial shrinkage can be woven into a fabric and then further shrinkage effected, thus giving a tighter weave. 15

The present invention is also applicable to the twist-setting of Nylon yarn in which a minor proportion (less than 50%) of the filaments is composed of other materials than Nylon, for example, cotton, regenerated cellulose, cellulose acetate, etc. The term "Nylon yarn," therefore, includes all yarns in which at least 50% of the filaments or fibers are composed of Nylon. 20

By this invention, there is now provided a method of setting the twist in a yarn so that it will run smoothly in subsequent textile operations such as knitting and weaving without the danger of snarls and loops due to the twist liveliness. At the same time, the twist-setting is accomplished without the danger of so setting the yarn itself that the fabric subsequently made from the yarn would be unsatisfactory, for reasons such as laciness or poor stitch formation, either of which is readily discernible by the 25 knitter.

Another advantage of this invention is that the twist liveliness is reduced more than it is when the yarn is set by means of steam without permitting shrinkage, even if the matter of yarn-set is completely ignored. For example, it is very difficult to set properly a twist of 50 turns per inch in 30-denier yarn according to the prior art procedure. It can be easily and successfully set according to this invention. Since, by this 30 invention, the yarn does not become set, it is a very important aspect.

Since it is obvious that many changes and modifications can be made in the above-described details without departing from the nature and spirit of the invention, it is to be understood that the invention is not to be limited to the details described herein except as set forth in the appended claims. 35

I claim:

1. The process of twist-setting a Nylon yarn to reduce the twist-liveliness thereof which comprises subjecting said yarn to a hot, wet treatment involving a temperature between 135° F. and 190° F. and a relative humidity in excess of 50% while maintaining the yarn under sufficiently low tensioning conditions to permit the same to shrink.

2. The process of twist-setting a Nylon yarn to reduce the twist-liveliness thereof which comprises subjecting said yarn to an atmosphere having a temperature between 135° F. and 190° F. and a relative humidity in excess of 50% while maintaining the yarn under sufficiently low tensioning conditions to permit the same to shrink.

3. The process of twist-setting a Nylon yarn to reduce the twist-liveliness thereof which comprises subjecting said yarn to a hot, wet treatment involving a temperature between 135° F. and 190° F. and a relative humidity in excess of 50% while maintaining the yarn under tensioning conditions not to exceed 0.66 gram per denier.

4. The process of twist-setting a Nylon yarn to reduce the twist-liveliness thereof which comprises subjecting said yarn to an atmosphere having a temperature between 135° F. and 190° F. and a relative humidity in excess of 50% while maintaining the yarn under tensioning conditions not to exceed 0.66 gram per denier.

5. The process of twist-setting a Nylon yarn to reduce the twist-liveliness thereof which comprises subjecting said yarn to an atmosphere having a temperature between 135° F. and 190° F. and a relative humidity between 85% and 100% while maintaining the yarn under tensioning conditions not to exceed 0.66 gram per denier.

6. The process of twist-setting a Nylon yarn to reduce the twist-liveliness thereof which comprises subjecting said yarn to an atmosphere having a temperature between 170° F. and 190° F. and a relative humidity in excess of 50% while maintaining the yarn under tensioning conditions not to exceed 0.66 gram per denier.

7. The process of twist-setting a Nylon yarn to reduce the twist-liveliness thereof which comprises subjecting said yarn to an atmosphere having a temperature between 170° F. and 190° F. and a relative humidity between 85% and 100% while maintaining the yarn under tensioning conditions not to exceed 0.4 gram per denier.

8. As a new article of manufacture, a Nylon yarn produced in accordance with the process of claim 1.

9. As a new article of manufacture, a Nylon yarn produced in accordance with the process of claim 3.

JOHN BLANCHARD MILES, JR.